

## UNITED STATES PATENT OFFICE

2,181,111

## METHOD FOR THE PRODUCTION OF METALLIC PRINTING PLATES OR CYLINDERS

Josef Horn, Dresden, Germany, assignor of fifty  
per cent to Erich Weber, Dresden, GermanyNo Drawing. Application May 27, 1936, Serial No.  
82,645. In Germany May 29, 1935

3 Claims. (Cl. 41—41.5)

This invention relates to a method for the production of metallic printing plates or cylinders comprising a plurality of layers, for book printing or for relief printing to obtain correct tone values or for printing from rollers prepared with the use of a screen.

There are already known printing plates or blocks comprising several metallic layers, as, for example, for book printing, e. g., zinc blocks or copper plates or cylinders for intaglio printing.

In order to increase the resistance to wear of such known printing plates, after the picture to be printed was applied thereto and finally cast or etched, such plates were nickel-plated or chromium-plated.

In the case of printing works or chemigraphical works which do not have their own metal electro-depositing plants, the cast or etched printing plates are first brought to so-called galvanoplastic installations, in order that the printing plates or cylinders may there be nickel-plated, chromium-plated or coated with zinc. This is a time-absorbing and expensive operation for printing works. Further, etched printing plates or cylinders which are subsequently provided with a metallic coating suffer from the drawback that with fine mesh autotypes the dots contract in consequence of the subsequently applied metallic deposits and affect unfavourably the truth to tone of the picture.

There are also already known multi-layer metallic printing plates or blocks in which, for example, a metallic layer is applied by metal atomisation or metal spraying to a base of copper or nickel.

The metallic layers produced by metal spraying on nickel or copper plates serve only to provide on such plates a porous grain adapted for retaining moisture, but not for etching high or deep a picture applied to the layer formed by metal atomisation.

If a picture is applied to one of the known metal bases and subsequently there is sprayed thereon a metallic layer which then is again dissolved at the printing areas, then in this case the truth to tone of the printed picture will be defective, because by the subsequently applied metallic spray, according to experience, a picture with the finest mesh with a sharpness true to the original is not obtained.

Bases consisting of iron, steel or other hard metal suffer from the drawback that in consequence of their hardness and slight flexibility they are very difficult to apply to printing cylinders of small diameter such as are common in

recent rotary printing machines. Further, iron and steel printing plates or blocks which come from the rolling mill have not such a uniform continuous smooth and close surface as is necessary for printing plates, even if the iron or steel bases are ground or polished before application of the metallic coatings. The treatment would also so increase the cost of the bases that they could not be economically used in the printing industry.

In another known printing plate the base also consists of steel which is plated with silver, nickel or copper. It is evident that these coatings do not serve to render the picture carrier more durable, because the steel base is much harder than the coating. They are rather intended to cause a chromate layer to adhere better. Also these steel bases suffer from the drawback of being difficult to bend and work on. Reference may also be made to a known metallic printing plate (mercury) with several metallic layers for planographic printing, where the upper layer applied to an iron basis consists of nickel which is etched through at the non-printing areas down to a copper layer which is then caused to form an amalgam. Apart from the fact that mercury printing plates have not been approved in practice, because they constitute a danger to health, and because the amalgamated copper faces repel the ink in a very defective manner, such printing plates have nothing in common with the subject of the application as they are planographic printing plates, while the subject of the application is concerned with printing plates having the inked areas in relief. The mercury printing plates are referred to only for the purpose of explaining the state of the art.

According to the invention the above mentioned drawbacks are avoided, and in metallic printing plates or blocks for book printing and for relief platen printing there is obtained a very durable picture carrier, true to tone value, with easy flexibility of the printing plate. In relief printing plates according to the invention, besides wear-resistant picture carriers of correct tone value and with the maximum ease of flexibility of the plate, there is obtained easy and satisfactory repulsion of the ink at the non-printing areas. This result is realised in that on a base of zinc, cadmium, tin, suitable light metals such as aluminium, magnesium or alloys thereof, for example, on zinc or aluminium plates, depending on the printing work to be effected, there is or are firmly superimposed one or more layers of copper, brass, tombac, tin, lead, aluminium, nickel, iron, 50

steel, manganese, chromium, alpaca, silver or alloys thereof, for example electrolytically or chemically, before the picture to be printed is transferred to the metallic layer which carries the picture, and the non-printing areas are deepened, etched, engraved or shaved. In this case the upper metallic layer or layers may be etched through, engraved or shaved at the non-printing areas. With relief printing plates this is desirable because then the underlying base, for example, one of zinc, can be readily made ink-repellant in manner known per se with a thin etch and water or aqueous solution.

A further very good example of such easily bendable relief printing plate with a picture carrier of great resistance to wear and correctness of tone value consists in a base plate of aluminium which is provided with one or more thin coating layers of copper or copper alloy. The picture is transferred in manner known per se to the upper cuprous carrier which is then etched away at the non-printing areas with dilute nitric acid, so that at these areas the aluminium or aluminium alloy or a thin metallic intermediate layer thereabove is caused wholly or almost wholly to appear. With suitable previous treatment these areas do not take up ink, but only the durable, copper-containing picture-carrier in relief is inked. As dilute nitric acid attacks only the copper alloy, but notoriously does not attack aluminium, it is impossible to effect too deep etching of the vacant points.

The correctness of tone value of the original, for example, of the negative, which is copied on the upper copper-containing layer is thus maintained in the cuprous picture carrier etched in relief.

In these examples the printing plates thus comprise bases of the easily flexed metals, zinc or aluminium, and the upper metallic coating or picture-carrying layer consists of hard wear-resistant metal, for example, copper or copper alloy. By etching away the upper metallic layer at the vacant points there is obtained a relieved cuprous picture, correct to tone, on an easily flexed and readily worked base plate. Between the base plate of zinc or aluminium and the upper metallic layer of copper or copper alloy there may naturally also be interposed the other metallic layers or some of the previously mentioned metallic layers.

Printing plates produced by the method just described present also the advantage that now also the offset printer can print with durable metallic original etchings of the correct tone value, which previously only the book printer was able to do.

To print with metallic wear-resistant original etched relief printing plates in order to produce offset printing similar to that of book printing has been for a long time the desire and aim of the offset printer. By the invention account is taken therefore of a long felt want.

A similar good example is realised if there is applied to a light metal base, for example an aluminium plate by fusion a thin iron layer which is deeply etched at the points free from the picture. Also in this case there is obtained a very durable relief picture carrier. This example can be used both for book-printing as also for offset relief printing.

Reference is still made to a further desirable example of a printing plate consisting of multiple layers of metal for book printing or for relief printing. In this case the base consists of suit-

able light metal, for example an aluminium plate. To this plate there is applied, for example chemically and by immersion, a thin layer of zinc or cadmium, and thereon there is superimposed a layer of copper alloy, for example, brass. The picture is then transferred in manner known per se to this brass layer, which is deeply etched at the points free from the picture or is etched through down to the zinc or cadmium layer or down to the light metal base. The intermediate layer of zinc or cadmium ensures perfect adhesion of the brass layer to the light metal base. Further, the said intermediate layers ensure uniform smooth continuous closeness of the brass layer. For fine mesh autotypes for offset printing this is a great advantage.

There may also be obtained a good example if to a base of zinc or other suitable light metal base there is applied a layer of tin, lead or amalgam and there is superposed on said layer a layer of copper alloy, for example a brass layer, and the points free from the picture are completely or almost completely etched away. The iron or tin or lead or amalgam layer enters into such a close combination with the light metal base which is exposed substantially throughout the non-printing areas and which in offset printing repels the ink very well at these areas.

It may also be mentioned that if on a base of zinc, cadmium, aluminium, tin or alloys thereof several metal layers are superimposed, such layers may consist of different metals; for example, on a zinc base there may first be superimposed a copper layer and then a silver layer. The transfer of the picture to the picture carrier may be effected by copying, printing, drawing, etc.

Instead of elemental metal layers also metal oxide layers may be electrolytically formed on a suitable light metal base such as aluminium or magnesium or alloys thereof, and then the picture may be applied to such metal oxide layers and made ready for printing in the manner already described.

An important advantage is realised if the base of light metal is somewhat roughened or grained electrolytically and then the other metal layers are applied thereto. If the covering metal layer or layers is etched away at the points free from the picture down to the electrolytically grained light metal base there is realised perfect retention of moisture, which is advantageous for offset printing.

Printing plates according to the invention may be provided not only on the front side but also on the rear side with the aforesaid metal covering layers, whereby an economic advantage is realised by saving of material, because both sides of such printing plates can be used.

In view of the fact that many of the metallic layers mentioned in the foregoing description must be etched with somewhat stronger acid solutions than are commonly necessary in che-migraphy for zinc, it is recommended not to treat with bichromated gelatin or albumen the light-sensitive layer which lies on the upper metallic layer and on which the picture is copied, but to use a so-called copying lacquer which is developed by means of alcohol. The subsequent removal of the copying lacquer may be assisted by solvents, for example, spirit.

In order to effect better adhesion to one another of the metallic layers it is important that they should not be polished before another layer is superimposed thereon. Also the uppermost

metallic layer need not be polished and ground before the light-sensitive layer or the picture is applied to the upper metallic layer.

6 The said metallic covering layers may not only be produced electrolytically or chemically but also by a metal spraying process or by hot rolling of copper on aluminium or by other methods.

10 As in offset printing works mainly plates of large area are used, the electrolytic application 10 of the metal layers with the necessary uniform thickness presents certain difficulties with large forms, in respect that the layer deposited on the printing plate is finer in the middle than at the edges, it is recommended in such cases to use 15 known devices such as filters which render it possible to obtain a uniform layer.

Further, it is recommended in the galvanic application of the layer or layers of copper, brass, 20 tombac, tin, lead, aluminium, nickel, chromium, 20 alpaca, or silver on a base of zinc, cadmium, aluminium, tin or alloys thereof to use alkali cyanide baths, because these ensure a greater 25 closeness and fineness of the grain of the electrolytic deposit which is advantageous for the metallic picture-carrying layer with the use of fine mesh drawings.

It may be mentioned also that printing plates according to the invention may be used both for direct printing and also for indirect or offset 30 printing.

I claim:

1. The method of producing metallic printing plates or cylinders for relief printing, which comprises superimposing upon a pliant ground plate of light metal selected from the group consisting of aluminium, magnesium and alloys thereof, at least one intermediate layer of a metal selected from the group consisting of zinc, cadmium and alloys thereof, superimposing on said intermediate layer or layers at least one layer of heavy wear-resistant metal characterized by an ability to carry printing ink and selected from the group consisting of copper, brass, tombac, chromium, nickel, alpaca, silver, steel and alloys thereof, and removing all of the metal 15 layers superimposed on the ground plate at the non-printing areas to such an extent that the top surface of the ground plate is exposed.

2. The method of producing metallic printing plates or cylinders for relief printing as set forth 20 in claim 1 in which the surface of the base plate is grained by electro-chemical treatment prior to the superimposition of the intermediate layer.

3. The method of producing metallic printing plates or cylinders for relief printing as set forth 25 in claim 1 in which the hard wear-resistant surface layer is deposited on the intermediate layer electrolytically from an alkali cyanide bath.

JOSEF HORN. 80